# EUROPEAN PATENT SPECIFICATION

(11) **EP 0 699 774 B1**
(45) Date of publication and mention of the grant of the patent: **20.10.1999**
(21) Application number: 95112050.0
(22) Date of filing: 01.08.1995
(51) Int. Cl.: C22C 38/04, C22C 38/44

(54) **Steels for monobloc tyres for railways and the like**
Stahl für Ein-Stück-Radreifen für Eisenbahnen oder ähnliches
Acier pour roues monoblocs pour chemins de fer et similaire

(30) Priority: 09.08.1994 IT MI941729
(43) Date of publication of application: 06.03.1996
(73) Proprietor: LUCCHINI SIDERURGICA S.p.A., 20121 Milano (IT)
(72) Inventor: Amici, Giampiero, I-24060 Sovere (IT); Ghidini, Andrea, I-24063 Castro (IT)
(74) Representative: Lecce, Giovanni

(56) References cited:
- DE-C- 3 446 794
- US-A- 4 348 800
- US-A- 4 975 041
- DATABASE WPI Week 7608 Derwent Publications Ltd., London, GB; AN 76-24043X & JP-A-51 002 616 (NIPPON STEEL CORP.KK) , 10 January 1976
- PATENT ABSTRACTS OF JAPAN vol. 014 no. 363 (C-0746) ,7 August 1990 & JP-A-02 133544 (NKK CORP) 22 May 1990,

## Description

This invention relates to a steel, utilizable for the fabrication of monobloc tyres for railways, tramways and underground railways.

It is known that one of the more critical problems in the field of rolling stock is constituted by the phenomenon of tyre fluting, which is a phenomenon of local deterioration of the rolling surface of rim, which, following localized wear, transforms in time its circular starting profile into a multiside polygonal profile.

During the running of the vehicle, such deterioration becomes a source of noise and, in order to restrain the sound emission within the limits provided for by the law, it is necessary to perform frequent profile grindings on the traditional materials used at present, in order to restore the original circular profile, which involves high costs and consumptions.

Object of this invention is to obviate the aforementioned drawbacks.

In its more general aspect, this invention allows to reach this object through the utilization, for the fabrication of monobloc railway tyres, of a C-Mn-Mo steel in which small amounts of elements (oligoelements) have been added comprising B, Zr, Nb, V and Al. The contemporaneous presence of such oligoelements, in well defined ratios relatively to one another and to the other elements comprised in the steels, allows to realize a synergetical activity which allows to obtain a good hardening, necessary to reach a remarkable hardness and wear resistance, higher than those of the traditional steels used at present for railway tyres, preserving at the same time toughness.

The composition is shown in the following table, where, besides oligoelements, also all the other elements comprised are indicated, stressing for some of them the extreme minimum and maximum percent contents foreseen.

| MICROALLOYED STEEL FOR MONOBLOC TYRES |
|---|
| 0.43 - 0.45 |
| ≤0.005 |
| ≤0.015 |
| 0.73 - 0.78 |
| ≤0.10 |
| 0.20 - 0.25 |
| 0.40 - 0.45 |
| ≤0.25 |
| 0.30 - 0.35 |
| ≤0.020 |
| ≤0.025 |
| ≤0.010 |
| 0.0010 - 0.0018 |
| 0.015 - 0.020 |
| 0.025 - 0.030 |
| 0.03 - 0.05 |

In the case of micro-alloyed steel for monobloc railway tyres, the following mechanical properties are ensured in the tyre plate and the rim crown.

| | Side plate | Rim crown |
|---|---|---|
| Ultimate tensile strength (N/mm2) | ≤850 | 940-1020 |
| Yield point (N/mm2) | | ≥700 |
| Elongation (%) | ≥15 | ≥14 |
| Striction (%) | ≥45 | ≥40 |
| CHARPY U resilience temp. = 20°C (Joule) | | ≥20 |

Said monobloc tyres undergo a differential hardening treatment in a suitable plant having known characteristics. Such heat treatment comprises the following steps:
- NORMALIZATION by heating at 870-930°C and following maintenance for 2-4 hours at such temperature, followed by spontaneous air cooling up to room temperature.
- ROUGH MACHINING;
- AUSTENIZITING by heating at 870-900°C and following maintenance for 2-4 hours at such temperature, followed by cooling in the differential hardening plant;
- TEMPERING through heating at 500-540°C, and following maintenance for 8-12 hours at such temperature, followed by spontaneous air cooling up to room temperature.

The tempering temperature of 500-540°C ensure, also in this case, that high toughnesses are reached and reduces the problems of surface hardness decline during shoe braking.

Also the conditions that promote wear resistance throughout the life of the monobloc tyre and the good homogeneity of the rolling surface hardness are ensured.

## Claims

1. A steel for monobloc tyres for use on railways, tramways and underground railways consisting of a C-Mn-Mo type steel micro alloyed with B, Zr, Nb, V and Al, which steel comprises the following elements in percent by weight:
| | |
|---|---|
| C | 0.43 - 0.45 |
| S | ≤ 0.005 |
| P | ≤ 0.015 |
| Mn | 0.73 - 0.78 |
| Cr | ≤ 0.10 |
| Ni | 0.20 - 0.25 |
| Mo | 0.40 - 0.45 |
| Cu | ≤ 0.25 |
| Si | 0.30 - 0.35 |
| Sn | ≤ 0.020 |
| As | ≤ 0.025 |
| Ti | ≤ 0.010 |
| B | 0.0010 - 0.0018 |
| Zr | 0.015 - 0.020 |
| Nb | 0.025 - 0.030 |
| V | 0.03 - 0.05 |
balance Fe apart from impurities.

2. A monoblock tyre for railways, tramways and underground railways made by the steel according to claim 1 and comprising a side plate and a rim crown which, after a differential hardening treatment comprising:
- normalization by heating at 870 - 930°C for 2 - 4 hours and spontaneous air cooling up to room temperature;
- rough machining;
- austeniziting by heating at 870 - 900°C for 2 - 4 hours and cooling in a differential hardening plant ;
- tempering by heating at 500 - 540°C for 8 - 12 hours and spontaneous air cooling up to room temperature, exhibit the following mechanical properties:
| Properties | Units | Side plate | Rim crown |
|---|---|---|---|
| Ultimate tensile strength | N/mm² | ≤ 850 | 940 - 1020 |
| Yield point | N/mm² | | ≥ 700 |
| Elongation | % | ≥ 15 | ≥ 14 |
| Striction | % | ≥45 | ≥ 40 |
| CHARPY U resilience (temp. = 20°C) | Joule | | ≥ 20 |

## Patentansprüche

1. Stahl für einstückige Reifen zur Verwendung bei Zügen, Strassenbahnen und Untergrundbahnzügen, der aus einem mit B, Zr, Nb, V und Al mikrolegierten C-Mn-Co-Typ Stahl besteht, dadurch gekennzeichnet, daß er folgende Elemente in Gewichtsprozent umfaßt:
| | |
|---|---|
| C | 0.43-0.45 |
| S | ≤ 0.005 |
| P | ≤ 0.015 |
| Mn | 0.73- 0.78 |
| Cr | ≤ 0.10 |
| Ni | 0.20 - 0.25 |
| Mo | 0.40 - 0.45 |
| Cu | ≤ 0.25 |
| Si | 0.30 - 0.35 |
| Sn | ≤ 0.020 |
| As | ≤ 0.025 |
| Ti | ≤ 0.010 |
| B | 0.0010 - 0.0018 |
| Zr | 0.015 - 0.020 |
| Nb | 0.025 - 0.030 |
| V | 0.03 - 0.05 |
Rest Fe abgesehen von Verunreinigungen.

2. Ein aus dem Stahl nach Anspruch 1 hergestellter einstückiger Reifen für Züge, Strassenbahnen und Untergrundbahnzüge, der eine Seitenplatte und einen Felgenkranz umfaßt, die nach einer Differential-Härtungsbehandlung umfassend:
- Normalisieren durch Erwärmen bei 870 - 930 °C für 2 - 4 Stunden und spontane Luftkühlung bis Zimmertemperatur;
- Grobbearbeiten;
- Austenitisieren durch Erwärmen bei 870 - 900°C für 2 - 4 Stunden und Kühlung in einer Differential-Härtungsanlage;
- Tempem durch Erwärmen bei 500 - 540°C für 8 - 12 Stunden und spontane Luftkühlung bis Zimmertemperatur,
folgende mechanische Eigenschaften aufweisen:
| Eigenschaften | Einheiten | Seitenplatte | Felgenkranz |
|---|---|---|---|
| Absolute Biegefestigkeit | N/mm² | ≤ 850 | 940 - 1020 |
| Streckgrenze | N/mm² | | ≥ 700 |
| Dehnung | % | ≥ 15 | ≥ 14 |
| Striktion | % | ≥45 | ≥ 40 |
| CHARPY U Elastizität (Temp. = 20°C) | Joule | | ≥ 20 |

## Revendications

1. Acier pour bandages monoblocs destinés à être utilisés sur des voies ferrées, des voies de tramways et de métro, constitué par un acier du type à C-Mn-Co, allié à des dispersoïdes comprenant B, Zr, Nb, V et Al, caractérisé en ce qu'il comprend les éléments suivants, en pourcentage en poids :
| | |
|---|---|
| C | 0,43 - 0,45 |
| S | ≤ 0,005 |
| P | ≤0,015 |
| Mn | 0,73 - 0,78 |
| Cr | ≤ 0,10 |
| Ni | 0,20 - 0,25 |
| Mo | 0,40 - 0,45 |
| Cu | ≤0,25 |
| Si | 0,30 - 0,35 |
| Sn | ≤ 0,020 |
| As | ≤ 0,025 |
| Ti | ≤ 0,010 |
| B | 0,0010 - 0,0018 |
| Zr | 0,015 - 0,020 |
| Nb | 0,025 - 0,030 |
| V | 0,03 - 0,05 |
le reste étant constitué de Fe, impuretés non comprises.

2. Bandage monobloc pour voies ferrées, voies de tramways et de métro, réalisé avec l'acier selon la revendication 1 et comprenant une plaque latérale et un bombé de jante qui, après un traitement de trempe différentielle comprenant :
- une normalisation par chauffage pendant 2 à 4 heures à 870-930°C et refroidissement spontané à l'air jusqu'à la température ambiante ;
- un ébauchage ;
- une austénitisation par chauffage pendant 2 à 4 heures à 870-900°C et refroidissement dans une installation de trempe différentielle ;
- un trempage par chauffage pendant 8 à 12 heures à 500-540°C et refroidissement spontané à l'air jusqu'à la température ambiante, présentent les caractéristiques mécaniques suivantes :
| Propriétés | Unités | Plaque latérale | Bombé de jante |
|---|---|---|---|
| Résistance à la rupture | N/mm² | ≤ 850 | 940 - 1020 |
| Limite d'allongement | N/mm² | | ≥ 700 |
| Allongement | % | ≥ 15 | ≥ 14 |
| Striction | % | ≥45 | ≥ 40 |
| Résilience Charpy avec entaille en U (temp. = 20°C) | Joule | | ≥ 20 |
